

April 15, 1958

G. R. MEYERS ET AL

2,830,913

CARBONACEOUS MOLDING MATERIAL FOR FOUNDRY OPERATIONS

Filed Oct. 11, 1955

4 Sheets-Sheet 1



Fig. 1

G. Roland Meyers  
Everett G. Gentry Inventors  
Small, Dunham & Thomas  
By Lee A. Strombeck Attorney

April 15, 1958

G. R. MEYERS ET AL

2,830,913

CARBONACEOUS MOLDING MATERIAL FOR FOUNDRY OPERATIONS

Filed Oct. 11, 1955

4 Sheets-Sheet 2



4



R4

Fig. 2

G. Roland Meyers  
Everett G. Gentry Inventors  
Small, Dunham & Thomas  
By Lee A. Trimble Attorney

April 15, 1958

G. R. MEYERS ET AL

2,830,913

CARBONACEOUS MOLDING MATERIAL FOR FOUNDRY OPERATIONS

Filed Oct. 11, 1955

4 Sheets-Sheet 3



Fig. 3

G. Roland Meyers  
Everett G. Gentry Inventors  
Small, Dunham & Thomas  
By Lee A. Thimbeck Attorney

April 15, 1958

G. R. MEYERS ET AL

2,830,913

CARBONACEOUS MOLDING MATERIAL FOR FOUNDRY OPERATIONS

Filed Oct. 11, 1955

4 Sheets-Sheet 4



Fig. 4

G. Roland Meyers  
Everett G. Gentry  
Small, Dunham & Thomas  
By Lee A. Steinbeck Attorney

1

2,830,913

**CARBONACEOUS MOLDING MATERIAL FOR FOUNDRY OPERATIONS**

Gustave Roland Meyers, Ann Arbor, and Everett G. Gentry, Lincoln Park, Mich., assignors to ESSO Research and Engineering Company, a corporation of Delaware

Application October 11, 1955, Serial No. 539,778

8 Claims. (Cl. 106—38.9)

The present invention relates to an improved carbonaceous material for molding metals. It more particularly pertains to an improved metals casting composition comprising fluid coke and a compounding material, for the formation of molds and cores used to cast articles of metal, including ferrous and non-ferrous metals and alloys thereof.

It has been discovered that fluid coke having less than 7 wt. percent sulfur serves as a superior metals casting material, and can be used to replace sand in molds and cores either partially or, more preferably, entirely. More specifically, this invention proposes that fluid coke of low sulfur content, by itself or in an admixture with sand, serves as an excellent material to form green, dried and baked molds, green and baked cores, mold facings, shell molds and cores, and the like. Fluid coke is an ideal metals casting material because it is carbonaceous, available in large quantities, and has a natural particle size similar to sand.

Superior results are obtained by using fluid coke as a metals casting material in that the articles cast have truer dimensional accuracy, smoother surface finish and require lesser cooling times. Because the thermal expansion of fluid coke is considerably less than that of conventional foundry sands, castings may be made with risers that are substantially reduced in size. In some cases the risers may be eliminated. Thus, more castings may be obtained from a melt and the amount of metal that must be recycled to the cupola for remelting is substantially reduced. Another advantage of fluid coke is that it is not "wetted" by molten iron because it is carbonaceous. This produces a smoother metal surface, and tends to prevent metal penetration and veining.

The hydrocarbon oil fluid coking process has recently been introduced into petroleum refinery operations. In this fluid coking process, an oil, usually a low value heavy residual oil, is converted by pyrolysis to relatively lighter hydrocarbons and coke by contact with finely divided heat carrying solid particles maintained at a temperature in the range of 850° to 1500° F. or above. The heat carrying solids are preferably maintained as a fluid bed in a coking zone, but the process can be carried out in a transfer line. The coke produced by the pyrolysis deposits on the fluidized solids, layer by layer, and becomes a part thereof. Although some of the coke produced by the cracking may be consumed by burning to supply heat in the coking process, a substantial amount is removed as by-product. The heat carrying solids normally used are coke particles produced by the process such that the by-product coke is of uniform composition. The by-product fluid coke produced has a high percentage of carbon with an ash and sulfur content characteristic of the oil feed stock.

The particle size of the heat carrying solid used in the coking process is in the range of about 18 to 400 U. S. sieve number, with the median particle size normally being in the range of 45 to 70. The by-product coke is of about the same size. This unique by-product coke is character-

2

ized by its spherical or ovoid shape, laminar structure, high density and hardness, and differs substantially from the cokes produced by the pyrolysis of hydrocarbonaceous solids and oils by other processes. The term "fluid coke" is intended to include the solid product of the fluid coking process, i. e., the by-product coke or "raw" fluid coke, besides the treated forms of the raw fluid coke, described below.

It has now been discovered that fluid coke as produced, but preferably raw fluid coke that has been pretreated, serves as an excellent metals casting material to form molds, cores, and mold and core washes. Fluid coke is a unique carbonaceous metals casting material because it is more nearly equivalent to sand in particle shape, hardness and density than any other carbonaceous material heretofore commercially available.

The preferred pretreatment of fluid coke comprises calcination and/or desulfurization to decrease its volatile matter and sulfur content, and to increase its density. The product so obtained by this pretreatment is herein-after referred to as calcined fluid coke. Although desulfurization treatment of raw fluid coke normally results in calcination of the coke, it is not necessarily always true and the term "calcined fluid coke" herein used, includes fluid coke that has only been desulfurized.

Calcination of the raw fluid coke to primarily increase its density and decrease its volatile matter content may be carried out by any conventional method. Generally, calcination of fluid coke simply involves heat soaking at relatively high temperatures, e. g., 1800° F. or above, for a suitable period of time. This is preferably done separate from the coking process, but may be carried out within the process, as by segmenting the burner used to heat fluid coke so as to form a special high temperature zone from which the by-product coke can be withdrawn. The calcination or heat soaking may be carried out while the fluid coke is in the form of a fixed, gravitating or fluid bed. A preferred method of calcination is to quickly heat the raw fluid coke up to about 2400° to 2800° F. by direct contact with high temperature flue gases or products of combustion, and then quickly separating the heated coke from the gases. The coke so heated is then maintained as a gravitating bed in a refractory lined soaking chamber for about one hour to complete the calcination. In this preferred manner of operating, volatile sulfur compounds, relatively undiluted with flue gases, can be recovered from the soaking zone.

It will be apparent to those skilled in the art that raw fluid coke can be calcined by repeated use in the casting process, and the term "calcination" is intended to include this. Thus, a small amount, say 5%, raw fluid coke can continuously be added to the reservoir of material used to form molds and/or cores in a foundry, and by repeated use become suitably calcined.

Desulfurization of raw fluid coke or of fluid coke that has been calcined can be accomplished in several ways. One preferred method is to oxidize the coke by fluidizing it with an oxygen containing gas at a temperature in the range of 600° to 1500° F. for a time sufficient to consume over 3 wt. percent of the fluid coke. An especially preferred method of desulfurization comprises this oxidation treatment followed by hydrogenation with a free hydrogen containing gas at temperatures above 1100° F. In some cases the fluid coke may be desulfurized without preliminary heat soaking, by contact with a desulfurizing gas such as hydrogen, ammonia, sulfur dioxide, etc. When using hydrogen it is preferred to maintain the temperature above 1100° F.; when using sulfur dioxide, the temperature is preferably maintained above 1800° F. Also, pressures of about 35 to 100 p. s. i. or above are useful during desulfurization.

Instead of treatment with a desulfurizing gas, the coke

can be desulfurized simply by a high temperature thermal treatment. Thus, at temperatures of about 2400°-2800° F., the sulfur compounds in coke can be broken down and driven off. At the lower temperature, several hours of heat soaking may be required to remove the sulfur.

In some uses it may be preferred, besides calcining the coke, to further pretreat it as by treatment with a solvent or by impregnating it with a suitable material such as water glass or finely divided graphite to decrease its porosity.

Fluid coke as removed from the fluid coking process, when coking the customary residual oil feed stocks, normally will have a sulfur content up to about 7 wt. percent or above. It is preferred to reduce the sulfur content if necessary, by the above treatments, to below about 7 wt. percent to prepare it for use in foundry operations because higher amounts of sulfur may produce intolerable amounts of noxious fumes. Raw fluid coke may, however, itself be used in casting operations as herein-after described.

To illustrate the change in properties that occurs during different treatments of raw fluid coke, Table I is presented. The examples given for each type of coke are based on raw fluid coke having an original median particle size of about 235 microns, obtained by the fluid coking of a Hawkins residuum having a gravity of 4.3° A. P. I., a Conradson carbon of 26 wt. percent, an initial boiling point of 882° F. (atmos. pressure equivalent), and a 10% point of 1010° F. The coking was at a temperature of about 1000° F.

The calcined fluid coke example is based on treating raw fluid coke as a gravitating fluid bed in an elongated vertical calcining chamber, at a temperature of about 2100° F. for a time up to about 15 hours.

The desulfurized fluid coke example was obtained by treating raw fluid coke as a gravitating moving bed in an externally heated elongated vertical silicon carbide brick-lined calcining tower. The coke was heated to a temperature up to about 2400° F. for a time of about 24 hours, in the presence of a small amount of nitrogen stripping gas.

TABLE I

|                                  | Examples       |                     |                         |
|----------------------------------|----------------|---------------------|-------------------------|
|                                  | Raw Fluid Coke | Calcined Fluid Coke | Desulfurized Fluid Coke |
| Size, A. F. S. No.               | 52             | 68                  | 75                      |
| True Density, grms./cc.          | 1.48           | 1.95                | 1.86                    |
| Bulk Density, lbs./gal.          | 9.6            | 9.6                 | 9.6                     |
| Moisture, wt. percent.           | 0.5            | nil                 | nil                     |
| Sulfur, wt. percent.             | 6.7            | 5.9                 | 2.0                     |
| Ash, wt. percent.                | 0.6            | 0.8                 | 0.3                     |
| Carbon, wt. percent.             | 88.3           | 97.7                | 97.7                    |
| Hydrogen, wt. percent.           | 1.8            | nil                 | nil                     |
| Volatile Matter, wt. percent.    | 5.6            | 0.2                 | nil                     |
| Base Permeability <sup>1</sup> . | 25/45          | 25/45               | 25/45                   |

<sup>1</sup> According to 6th ed., "Foundry Sand Handbook."

Generally speaking, calcination of fluid coke normally having a sulfur content of 1-12 wt. percent, will reduce its volatile matter content below about 1 wt. percent and sulfur content by 5-20%, and increase its true density above 1.7 grms./cc. Desulfurization will reduce sulfur content to below 3 wt. percent. It is preferred to use fluid coke having characteristics falling in these ranges, as superior results are obtained even over raw fluid coke.

Fluid coke, including raw, calcined, and calcined-desulfurized fluid coke, is preferably used as the principal constituent in molds, cores, washes, mold facing materials, mold backing materials, etc., replacing sand entirely, but can, however, be used in lesser amounts admixed with sand, or in minor amounts (0.5 to 25%) used as an additive, the term "metals casting material"

being intended to include all of these uses. Any type of mold and/or core can be made according to this invention including, for example, conventional green, air dried, baked, shell, sand spun, oil, cement and investment molds, and green, air dried, baked, shell, CO<sub>2</sub> process, and cement cores. The molds and cores may be formed either by hand ramming or with mechanical equipment. When reduced in particle size, fluid coke can serve as an ingredient in mold and core washes.

In the preparation of molds, cores, and washes, fluid coke is admixed with conventional additives or compounding materials customarily used in the preparation and shaping of molds and cores. By compounding materials it is meant to include conventional binders such as water, oils, compounded core oils, marine oils, iron oxide, drying oils, silica and wood flour, bentonite, dextrine, sea coal, cereal, clay, sugars, lignin sulfite, thermosetting and thermoplastic resins, pitch, rosins, etc.; to include conventional mold additives such as water, oils, resin, cereal, bentonite, clays, sea coal, iron oxide, water glass, silica and wood flours, water soluble binders, sand and clay; and to include conventional mold and core wash, paste and filler ingredients, such as water, graphite, plumbago, sea coal, resins, corn oil, molasses, clay, organic solvents, dextrine, bentonite, gelatin, zircon and silica flours, etc. Molds and cores made of fluid coke can be used to cast ferrous and non-ferrous metals and their alloys including gray, nodular and malleable iron, aluminum, magnesium, copper, lead, etc., and copper base and steel alloys.

Figure 1 through 4, showing various articles cast according to this invention, are presented to further clarify this discussion.

Calcined fluid coke used as a metals casting material results in a superior cast product. The castings possess truer surface dimensions and exterior and interior contours, and have a more perfect finish. Fewer casting defects result.

The relatively low thermal expansion of fluid coke, as compared to conventional molding and core sands, is a highly desirable characteristic. It results in fewer casting defects that are attributable to expansion-contraction forces developed in the mold and/or core by the heat of the metal during and shortly after pouring. Fluid coke has been found to be at least equivalent, if not superior, to zircon sand in this respect. A fluid coke mold has  $\frac{1}{10}$  to  $\frac{1}{4}$  of the expansion of a conventional sand mold. The relatively small thermal expansion of fluid coke and its more rapid heat transfer characteristics permit the casting of a metal using a smaller riser, or fewer risers, which substantially reduces the amount of metal that must be recycled. Fluid coke produces a good reducing atmosphere when pouring a mold, even when used as an additive.

The faster cooling obtained through the use of fluid coke permits shorter mold cooling times to be realized. When casting non-ferrous metals such as brass and aluminum, this higher rate of cooling results in castings having a finer grain size and structure than that normally obtained, which is highly desirable. It will be appreciated by those skilled in the art that the higher heat conductivity of fluid coke as compared to sand, appreciably decreases baking times and/or temperatures of baked molds and cores, and results in a more uniform baking.

Because fluid coke has a bulk density about 20% less than conventional sand, a lesser weight of material can be used, thereby decreasing handling costs. It has been found that when casting steels, there is a case hardening effect caused by the fluid coke which is desirable in some instances. With gray cast iron which is fully saturated with carbon, the carbonaceous material does not affect the casting. Because fluid coke is substantially pure carbon, molten iron does not tend to wet or adhere to it.

This greatly reduces or eliminates metal penetration, veining, etc., and improves surface finish. When conventional sand is used, iron silicate, a low melting slag and forerunner to veining, may be formed. This cannot happen with fluid coke.

Tests have shown that fluid coke when used in molds, does not suffer any substantial loss and may be reused. It has, in fact, been found that reused calcined fluid coke or shake-out fluid coke has some advantages because the previous use causes some further calcination and desulfurization of the coke, thereby improving its properties.

Generally, it is desired that the sulfur content of fluid coke be below 7 wt. percent because of the fumes created and/or to minimize the sulfur pick up on the surface of the casting. With ferrous metals, particularly gray cast iron, it is preferred to use fluid coke having a sulfur content below 3 wt. percent because a higher sulfur content may result in an appreciable formation of iron sulfide on the surface of the casting. This may cause undesirable cracking and hardening of the surface. In some instances, however, this may be an advantage, e. g., when the iron is compounded with manganese. The sulfur in the coke preferentially forms manganese sulfide, which imparts improved properties to the casting. With non-ferrous metals, the presence of sulfur also may not necessarily be detrimental, particularly in casting brass and aluminum. When casting magnesium, the raw fluid coke of high sulfur content may be preferred because sulfur is normally used as an inhibitor in mold and core mixtures in casting magnesium.

Generally speaking, it has been found that greater amounts of certain additives must be used when compounding green molds of fluid coke, while the amount of other types of additives normally used can be reduced or eliminated over that normally used with sand. For example, up to 50% more water may be used with fluid coke. When using oils, such as drying, marine, and/or conventional core oils, the amount of oil used is normally somewhat greater than that used with core sands because of the greater volume per weight of fluid coke. With molds and cores, it is preferred to fully temper the coke particles with water before adding a liquid binder.

The fluid coke is, of course, comminuted if necessary, either before or after calcination, and classified to obtain the proper size and size distribution needed in the particular casting process.

Tests have been conducted to determine the range of uses to which fluid coke may be applied. Gray cast iron, steel, bronze, (brass), and aluminum have been tested in commercial operation using raw, calcined, or calcined-desulfurized fluid coke to form green molds, shell molds and cores. The mold-forming and casting process used in some cases where those then being used to make commercial articles of manufacture. Fluid coke was used to replace in its entirety, and partially conventional molding sand. Tests were also conducted under more severe conditions of casting bronze, specifically bronze pump impellers, where zircon sand is used because of its low thermal expansion characteristics to obtain a good casting.

In all cases, calcined fluid coke was found to produce a casting equal, and more often superior, to the conventional cast product. Taking in account the different physical characteristics of fluid coke, the molding procedures used were substantially the same.

#### Example I

Fluid coke was used to form a cope and drag for the casting of a commercially manufactured pump head. The pump head of gray cast iron was cast in molds made of raw fluid coke, of calcined-desulfurized fluid coke, and of conventional molding sand. The properties of the raw and calcined coke are given in Table I. The particle size of the fluid coke and sand are given in Table II, and the composition and properties of the molds are given in Table III.

6  
TABLE II

| 5                 | U. S. Sieve No. | Raw Coke, Wt. Percent Retained | Calcined Coke, Wt. Percent Retained | Sand, Wt. Percent Retained |
|-------------------|-----------------|--------------------------------|-------------------------------------|----------------------------|
| 10                | 6               | 0.2                            | 0                                   | 0                          |
|                   | 12              | 0.2                            | 0.8                                 | 0                          |
|                   | 20              | 0.4                            | 1.0                                 | 0.2                        |
|                   | 30              | 0.2                            | 2.6                                 | 0.4                        |
|                   | 40              | 2.0                            | 3.6                                 | 3.8                        |
|                   | 50              | 32.2                           | 12.3                                | 17.0                       |
|                   | 70              | 43.8                           | 28.7                                | 34.4                       |
|                   | 100             | 15.6                           | 23.0                                | 30.2                       |
|                   | 140             | 3.4                            | 15.1                                | 8.8                        |
|                   | 200             | 1.4                            | 8.7                                 | 2.4                        |
| 15                | 270             | 0.2                            | 2.2                                 | 0.8                        |
|                   | Pan             | 0.2                            | 2.0                                 | 0.6                        |
| A. F. S. Fineness |                 | 52.7                           | 75                                  | 63                         |

<sup>1</sup> Clay.

TABLE III

| 25 |                                                                                                                                                                                                                                  | Raw Fluid Coke                           | Calcined Fluid Coke Mixture              | Conventional Sand Mixture                |
|----|----------------------------------------------------------------------------------------------------------------------------------------------------------------------------------------------------------------------------------|------------------------------------------|------------------------------------------|------------------------------------------|
| 30 | Composition: 1<br>Raw Fluid Coke, weight percent<br>Calcined Fluid Coke <sup>2</sup> do<br>Sand do<br>Mogul-Cereal Binder do                                                                                                     | 100                                      | 100                                      | 100                                      |
| 35 | Wheat Flour do<br>Wood Flour do<br>Western Bentonite do                                                                                                                                                                          | 1.2                                      | 1.2 approx.                              | 1.2                                      |
| 40 | Southern Bentonite do<br>Sea Coal do<br>Water do                                                                                                                                                                                 | 3.9                                      | 3.9 approx.                              | 2.9                                      |
| 45 | Physical Properties:<br>Green Permeability<br>Green Compressive Strength, p. s. i.<br>Deformation, percent<br>Hot Strength @ 1,500° F., p. s. i.<br>Hot Strength @ 2,000° F., p. s. i.<br>Thermal Expansion @ 1,500° F., in./in. | 130<br>5.4<br>0.027<br>107<br>2<br>3.003 | 35<br>3.3<br>0.022<br>395<br>20<br>0.004 | 120<br>5.6<br>0.018<br>92<br>18<br>0.022 |
| 50 | Mold Hardness, Cope<br>Mold Hardness, Drag<br>Pour Temperature, °F.                                                                                                                                                              | 70<br>75<br>2,580                        | 70<br>75<br>2,580                        | 55<br>75<br>2,540                        |

<sup>1</sup> This and subsequent tables are based on coke (and sand where applicable) as totaling 100 wt. percent, with all other ingredients being 45 wt. percent based on coke and/or sand.

<sup>2</sup> This is shake-out coke.

<sup>3</sup> In 3 min., then contracted to -0.024 in./in. in 12 min.

In subsequent tests it was noted that one-half hour after the pouring of the castings, when the molds were shaken out, the casting from the conventional mold was at cherry red heat while those from the fluid coke, both raw and calcined, were at black heat. This shows that fluid has a much higher heat conductivity which is desirable because it minimizes shrinkage of the casting.

55 Figure 1 shows the castings obtained from this test. The casting marked 8R is from the conventional sand mold, the one marked 8 is from the mold using raw fluid coke, and the one marked 9 is from the mold using calcined-desulfurized fluid coke. It is to be noted in the drawing that the riser, indicated by an arrow, attached to pump head #9 is not depressed or pipe while riser of the conventional mold shows piping. This illustrates that metal was drawn into the mold during the cooling process in the conventional mold because of the thermal expansion of the mold, and because of the slower cooling time. The riser from the calcined fluid coke mold is more uniform and does not display this piping. This illustrates that in some instances the riser may be eliminated and may, in most cases, be substantially reduced in size.

60 Under similar conditions, calcined fluid coke (not desulfurized), having a sulfur content of 5.9 wt. percent and volatile matter content of 0.2 wt. percent, was used to form a mold for a cast gray iron pump head. Molds 65 were cast using a riser and without a riser, using for com-

## Example IV

parison conventional sand molds. The castings were poured at 2620° F. The castings using only calcined fluid coke possessed a better surface smoothness than those from conventional sand molds, but not as smooth as those from calcined-desulfurized fluid coke. The calcined fluid coke without a riser produced a satisfactory casting.

Malleable cast iron can be cast as well as gray cast iron.

Steel was also cast in a pump head shaped mold. There was found to be a surface case hardening effect which in some cases may be desirable.

Sulfur prints were taken to determine the extent of sulfur pick up by the castings. In no case was it found to be detrimental as, for example, to interfere with subsequent machining, because the thickness of the sulfur-containing layer in the casting was minor. Sulfur pick up usually results in a negligible hardening of the surface.

## Example II

Fluid coke having a size distribution as in Table II was fabricated into the mold for the casting of bronze having the specification: Brass #165 "M"—USN—A. S. T. M. B30 alloy 2A—copper base ingots—A. S. T. M.—NIB 16541—bronze castings. Concurrently with casting of bronze in a calcined fluid coke mold, an identical casting was made in a conventional sand mold. The composition and properties of the molds are given in Table IV.

TABLE IV

|                                          | Calcined Fluid Coke Mixture | Sand Mixture |  |
|------------------------------------------|-----------------------------|--------------|--|
| Composition:                             |                             |              |  |
| Sand..... weight percent                 |                             | 100          |  |
| Calcined Coke..... do                    | 100                         |              |  |
| Southern Bentonite..... do               | 5.1                         | 4.8          |  |
| Pitch..... do                            | 1.0                         | 1.0          |  |
| Water..... do                            | 3.9                         | 3.4          |  |
| Physical Properties:                     |                             |              |  |
| Moisture, wt. percent.....               | 3.8                         | 3.3          |  |
| Green Permeability.....                  | 37                          | 52           |  |
| Green Compressive Strength, p. s. i..... | 4.7                         | 8.2          |  |
| Deformation, percent.....                | 0.021                       | 0.012        |  |
| Hot Strength @ 1,500° F., p. s. i.....   | 180                         | 180          |  |
| Hot Strength @ 2,000° F., p. s. i.....   | 6                           | 102          |  |
| Mold Hardness, Cope.....                 | 45                          | 75           |  |
| Mold Hardness, Drag.....                 | 55                          | 75           |  |
| Pour Temperature, ° F.....               | 2,250                       | 2,250        |  |

The resulting casting from the calcined fluid coke mold shown in the left side of Figure 2 had a smoother surface finish than the one produced in a conventional sand mold shown in the right side of Figure 2. What is more important, the grain structure of the bronze casting produced from the calcined fluid coke mold was considerably finer. This is a desired characteristic because it materially improves the machinability and strength of the casting.

## Example III

Fluid coke was used to form shell molds for casting a commercially produced aluminum drill housing, as shown in Figure 3. Calcined-desulfurized fluid coke of a particle size given in Table II was mixed with 6.1% of a commercial phenol resin binder and used to form the shell mold identified as number 10 in Figure 3, and 6.0% of the same resin was mixed with sand for the shell mold marked 10R. The cores used were made of sand and not of fluid coke. The casting produced with fluid coke molds had a better surface finish, metal grain structure, and dimensional design than castings produced by conventional shell molding methods. This example shows that superior results are obtained using fluid coke as a metals casting material when casting aluminum.

Calcined-desulfurized fluid coke was used by itself or mixed with zircon sand to make cores for a commercially produced bronze pump impeller requiring a high degree of perfection. Table V lists the compositions of the cores and of similar cores made from conventional zircon sand, and Table VI gives the properties of the cores. All cores, after baking in a rack oven at about 460° F. for 1½ hours, were coated with silica wash and dried for 30 minutes in a rack oven. The bronze was poured at 2075° F. simultaneously into molds having zircon sand cores and molds having fluid coke cores. The molds were conventional, bake, pitch-bonded molds.

TABLE V

|                                 | Conventional, Wt. percent | This Invention, Wt. percent |
|---------------------------------|---------------------------|-----------------------------|
| Zircon Sand.....                | 100                       |                             |
| Fluid coke through 60 mesh..... |                           | 38                          |
| Fluid coke through 8 mesh.....  |                           | 62                          |
| Mogul—Cereal Binder.....        |                           | 2.0                         |
| Core Oil.....                   | 0.5                       | 2.0                         |
| Water.....                      | 0.8                       | 2.0                         |

TABLE VI

|                                                | Conventional | This Invention |
|------------------------------------------------|--------------|----------------|
| Moisture, wt. percent.....                     | 0.8          | 7.0            |
| Dry Permeability.....                          | 39           | 39             |
| Tensile Strength, Lab.....                     | 368+         |                |
| Scratch Hardness, Lab.....                     | 98           |                |
| Tensile Strength, after 1½ hrs. at 500° F..... |              | 118            |
| Scratch Hardness, after 1½ hrs. at 500° F..... |              | 100            |

Figure 4 illustrates vertical cross-sections of the castings produced. The letter Z indicates a casting produced by using conventional zircon sand cores, and the letter C indicates a casting using fluid coke cores. As evidenced by Figure 4, the fluid coke core casting shows smooth internal surface and freedom from metal penetration. It was equal in all respects to casting "Z" and did not suffer the shrinkage void of casting "Z." This example shows that fluid coke can be used to make cores at least equal, if not superior, to zircon sand cores.

Cores comprising 25/75, 50/50, and 75/25 fluid coke to sand were made up and found to be satisfactory when compared to conventional cores.

An A. F. S. baked tensile core specimen, 1" thick, comprising 2% cereal, 2% oil, 4% water, 50% calcined fluid coke, and 50% core and sand was baked at 400° F. and peak strength was developed in less than 45 minutes. This illustrates the better heat conductivity of fluid coke because test cores of sand normally require a longer baking time.

The following Table VII presents preferred typical ranges of compositions that can be used to form green, baked oil-bonded and shell cores and molds, which are preferred applications of fluid coke.

TABLE VII  
COMPOSITION RANGES OF MOLDS AND CORES

|                 | Weight percent of— | Green   | Baked   | Shell |
|-----------------|--------------------|---------|---------|-------|
| Fluid Coke..... | 25-100             | 25-100  | 25-100  |       |
| Sand.....       | Balance            | Balance | Balance |       |
| Water.....      | <10                | <10     | <10     |       |
| Bentonite.....  | <10                |         |         |       |
| Cereal.....     | <4                 | <4      | <4      |       |
| Resin.....      |                    |         |         | <12   |
| Oil.....        |                    | <4      |         |       |

It will be appreciated by those skilled in the art that because of the carbonaceous nature of this new casting material, in many instances conventional additives such

as pitches, plumbago, graphite, and sea coal formerly compounded with molding sands may be dispensed with.

It can be seen that fluid coke results in a casting process that is more rapid and produces a casting of truer accuracy and superior surface characteristics, because it minimizes mold movement. One advantage accruing to fluid coke is that risers may be eliminated or substantially reduced in size, thus permitting foundries to approach 100% yield through minimizing remelting of risers. Other principal advantages of fluid coke are that it has a low thermal coefficient of expansion, and a higher heat conductivity when compared to sand, and is not wetted by molten iron.

Having described this invention, what is sought to be protected by Letters Patent is succinctly set forth in the following claims.

What is claimed is:

1. A metal molding composition consisting essentially of fluid coke, and a compounding material, said fluid coke having been produced by contacting a heavy petroleum oil coking charge stock at a coking temperature with a body of fluidized coke particles in a reaction zone wherein the oil is converted to product vapors and carbonaceous solids are continuously deposited on the coke particles, removing product vapors from the coking zone, heating a portion of the coke from the coking zone in a heating zone to increase the temperature of said fluidized particles, returning a portion of the heated coke particles from the heating zone to the coking zone and withdrawing coke product particles.

2. The composition of claim 1, wherein said fluid coke has a sulfur content below 7 wt. percent, a volatile matter content below 1 wt. percent, and a true density above 1.7 gms./cc.

3. An improved metals casting form which consisting

essentially of an admixture of calcined fluid coke and a compounding material formed to the desired shape.

4. The form of claim 3 wherein said admixture consisting essentially of from 25 to 100% fluid coke, the balance being sand, and said compounding material comprises under 10 wt. percent water and under 12% of a binder material.

5. The form of claim 3 wherein said compounding material is a binder, and said form is baked.

6. An improved metals molding and casting composition consisting essentially of fluid coke, sand, and a compounding material, said compounding material comprising water and a binding agent, and said composition being characterized as follows on a weight percent basis of total coke and sand:

25 to 100 weight percent—fluid coke, the balance being sand.

Less than 10 weight percent—water.

Less than 12 weight percent—binding material.

7. The composition of claim 6 wherein said fluid coke has a sulfur content of less than 7 weight percent.

8. An improved metals molding composition consisting essentially of sand, fluid coke, and a compounding material, the weight ratio of fluid coke to sand being not greater than 0.5.

References Cited in the file of this patent

UNITED STATES PATENTS

|    |           |             |       |               |
|----|-----------|-------------|-------|---------------|
| 30 | 1,871,315 | Gann        | ----- | Aug. 9, 1932  |
|    | 1,886,252 | Gann et al. | ----- | Nov. 1, 1932  |
|    | 2,218,781 | Baggett     | ----- | Oct. 22, 1940 |

FOREIGN PATENTS

|    |         |        |       |               |
|----|---------|--------|-------|---------------|
| 35 | 511,794 | Canada | ----- | Apr. 12, 1955 |
|----|---------|--------|-------|---------------|